

## CELLULOSE ACETATE SPINNING PROCESS

François J. Olmer, Morristown, N. J., assignor to Celanese Corporation of America, New York, N. Y., a corporation of Delaware

No Drawing. Application November 24, 1950,  
Serial No. 197,516

1 Claim. (Cl. 18—54)

This invention relates to filamentary materials and relates more particularly to a process for the production of filamentary materials having a basis of cellulose acetate or other organic acid ester of cellulose.

It is an important object of this invention to provide a process for the production of high tenacity filamentary materials having a basis of cellulose acetate or other organic acid ester of cellulose.

A further object of this invention is to provide an improved process for the production of filamentary materials wherein a solution of cellulose acetate or other organic acid ester of cellulose is spun into a coagulating medium comprising a latent solvent incapable of dissolving the cellulose ester, but capable of swelling it to a considerable extent.

A still further object of this invention is to provide an improved process for the production of filamentary materials wherein a solution of cellulose acetate or other organic acid ester of cellulose is spun into a coagulating medium comprising a mixture of carbon tetrachloride and methylene chloride.

Another object of this invention is to provide a process for the production of filamentary materials wherein a solution of cellulose acetate or other organic acid ester of cellulose is spun into a coagulating medium comprising a mixture of carbon tetrachloride and methylene chloride and the filamentary materials are passed, while still wet with the coagulating medium, into a saponification bath.

Other objects of this invention will be apparent from the following detailed description and claim.

In the production of filamentary materials having a basis of cellulose acetate or other organic acid ester of cellulose by the wet-spinning process, a solution of the filament-forming material in a suitable solvent is pumped or otherwise forced through a spinning jet, having at least one spinning orifice therein, into a liquid coagulating medium which causes the filament-forming material to coagulate or set and which extracts the solvent therefrom. It has previously been proposed to increase the tenacity of the filamentary materials produced in this manner by stretching said materials during the spinning operation while they are still in a relatively plastic state. In this way, it is possible to produce filamentary materials having tenacities of from 2 to 5 or more grams per denier. However, the increase in the tenacity of the filamentary materials is accompanied by a reduction in their elongation, so that it is difficult to weave, knit or otherwise process said high-tenacity filamentary materials into textile fabrics.

I have now discovered that by spinning a solution of cellulose acetate or other organic acid ester of cellulose into a coagulating medium comprising a latent solvent incapable of dissolving the cellulose ester, but capable of swelling it to a considerable extent, such as a mixture of carbon tetrachloride and methylene chloride, and stretching said filamentary materials while they are still in a relatively plastic state, it is possible to obtain products having both a high tenacity and a good elongation which may be converted without difficulty into textile fabrics. Thus, in accordance with the present invention a solution of cellulose acetate or other organic acid ester of cellulose is pumped or otherwise forced through a spinning jet, having at least one spinning orifice therein, into a coagulating medium comprising a mixture of the type specified above. The filamentary materials formed in this manner are stretched while they are still in a relatively plastic state,

following which they are dried to remove therefrom the coagulating medium. Filamentary materials prepared in this manner exhibit a tenacity of from 2 to 4 or more grams per denier coupled with an elongation of from 15 to 25% at the breaking point. The properties of the filamentary materials obtained with a given coagulating medium depend upon the composition of said medium and the extent to which said filamentary materials are stretched during their production, the higher the degree of stretch the higher the tenacity and the lower the elongation of the final product.

In carrying out the process of the present invention, a spinning solution or dope is prepared by dissolving cellulose acetate or other organic acid ester of cellulose in a suitable solvent such as, for example, acetone, acetone-water mixtures, 98:2% by weight or 95:5% by weight, preferably in an amount sufficient to yield spinning dope containing from about 18 to 28% by weight of the filament-forming material. The spinning dope, after being filtered to remove therefrom all solid impurities, is spun into a coagulating medium containing, for example, from about 10 to 25% by volume of carbon tetrachloride, the remainder being methylene chloride. As the spinning dope enters the coagulating medium, the filament forming material is caused to set or gel and the solvent is extracted therefrom by the coagulating medium. Other coagulating media that may be employed include, for example, dichloroethane and tetrachloroethane alone; ethylene chloride, alone, or admixed with carbon tetrachloride (95:5% by weight); chloroform admixed with carbon tetrachloride (80:20% to 90:10% by weight) and methylene chloride admixed with benzene, toluene, cyclohexane and the like.

While the filamentary materials are still in a relatively plastic state, they are stretched to increase their length by about 1000 to 5000%. The stretching may be effected by passing the filamentary materials over a number of rollers immersed in the coagulating medium, each successive roller having a higher peripheral speed than the preceding roller. Preferably, however, the stretching is effected by means of a positively driven roller which draws the filamentary materials from the coagulating medium at the proper speed. After the filamentary materials emerge from the coagulating medium they are dried, following which they may be twisted and wound onto a textile package or otherwise treated to prepare them for further use.

The coagulating medium is advantageously maintained at a temperature of from about 0 to 30° C. depending upon its composition. When the coagulating medium is employed at the higher temperatures within this range, say above about 25° C., the concentration of any cellulose ester solvent, such as methylene chloride, therein should be kept below the value at which excessive softening of the filamentary materials will take place, which, when multi-filament materials are being produced, may cause the individual filaments thereof to coalesce, one with the other.

To improve the tenacity and/or to modify the dyeing and other properties of the filamentary materials prepared in the manner set forth above, it is frequently desirable to saponify the cellulose acetate or other organic acid ester of cellulose, either partially or completely. While the saponification may be effected by treating the dried filamentary materials with a suitable saponification bath, it has been found that the saponification may be effected more rapidly and more uniformly by passing the filamentary materials through the saponification bath while they are still wet with the coagulating medium. Thus, the filamentary materials may be passed directly from one container holding the coagulating medium into another container holding the saponification bath, care being taken to avoid any substantial evaporation of the coagulating medium from the filamentary materials as said materials pass from one container to the other. A preferred method for effecting the saponification is to float a saponification bath immiscible with the coagulating medium on the coagulating medium so that the filamentary materials will pass through said saponification bath as they emerge from the coagulating medium. In this way,

the escape of the coagulating medium from the filamentary materials before they enter the saponification bath is substantially avoided and, in addition, the saponification bath acts to seal the coagulating medium from the atmosphere thereby minimizing the loss of said medium through evaporation. When the saponification has progressed to the desired extent, the filamentary materials are withdrawn from the saponification bath and are washed to remove therefrom the products of saponification and the saponification bath and dried, following which they may be twisted and wound onto a textile package or otherwise treated to prepare them for further use.

As the saponification bath there may be employed, for example, aqueous solutions of alkaline materials such as sodium hydroxide, potassium hydroxide or ammonium hydroxide, to which solutions there may be added buffering salts such as sodium acetate, potassium acetate or ammonium acetate to make more uniform the action of said baths.

The process of this invention will now be described specifically in connection with the production of filamentary materials having a basis of cellulose acetate, which is commercially the most important organic acid ester of cellulose at the present time. It may also be employed for the production of filamentary materials having a basis of other organic acid esters of cellulose, such as, cellulose propionate, cellulose butyrate, cellulose acetate propionate and cellulose acetate butyrate.

The following examples are given to illustrate this invention further.

*Example I*

Dope containing 26% by weight of cellulose acetate dissolved in acetone is spun into a coagulating medium containing 85% by volume of methylene chloride and 15% by volume of carbon tetrachloride maintained at a temperature of 25° C. The filamentary materials travel through said coagulating medium for a distance of 6 inches and are stretched to increase their length 1300%. Upon emerging from said medium the filamentary materials are dried and wound onto a spool at a rate of 70 meters per minute. The filamentary materials exhibit a tenacity of 4.30 grams per denier and an elongation of 23% at the breaking point.

*Example II*

Dope containing 25% by weight of cellulose acetate, having an acetyl value of 54.6%, calculated as acetic acid, dissolved in acetone, is spun into a coagulating medium containing 82.5% by volume of methylene chloride and 17.5% by volume of carbon tetrachloride maintained at a temperature of 25° C. The filamentary materials travel through said coagulating medium for a distance of 9 inches and are stretched to increase their length 2200%. The filamentary materials then travel through a 3 inch layer of 20% aqueous ammonium hydroxide which is floated upon the surface of the coagulat-

ing medium. Upon emerging from the coagulating medium, the filamentary materials are washed and dried and are then wound onto a spool at a rate of 81 meters per minute. The filamentary materials are partially saponified and have an average acetyl value of 48%, calculated as acetic acid, and exhibit a tenacity of 3.24 grams per denier and an elongation of 16.4% at the breaking point.

*Example III*

The process set forth in Example I is repeated, employing as a coagulating medium a mixture of 95% by weight of ethylene chloride and 5% by weight of carbon tetrachloride, and taking up the filamentary materials at a rate of 97 meters per minute. The filamentary materials exhibit a tenacity of 2 grams per denier and an elongation of 43% at the breaking point.

*Example IV*

The process set forth in Example I is repeated, employing as a coagulating medium a mixture of 82.5% by weight of methylene chloride and 17.5% by weight of cyclohexane, and taking up the filamentary materials at a rate of 68 meters per minute. The filamentary materials exhibit a tenacity of 3.5 grams per denier and an elongation of 22% at the breaking point.

It is to be understood that the foregoing detailed description is given merely by way of illustration and that many variations may be made therein without departing from the spirit of my invention.

Having described my invention, what I desire to secure by Letters Patent is:

Process for the production of filamentary materials which comprises spinning a solution containing 25% by weight of cellulose acetate having an acetyl value of 54.6% dissolved in acetone into a coagulating medium maintained at 25° C. and containing 82.5% by volume of methylene chloride and 17.5% by volume of carbon tetrachloride, stretching the filamentary materials to increase their length 2200% while they travel through said coagulating medium for a distance of 9 inches, then passing said filamentary materials through a 3 inch layer of 20% aqueous ammonium hydroxide which is floated on the coagulating medium to reduce the average acetyl value of the cellulose acetate to 48%, washing and drying the filamentary materials, and taking up the filamentary materials at a rate of 81 meters per minute.

References Cited in the file of this patent

UNITED STATES PATENTS

|    |           |                |       |               |
|----|-----------|----------------|-------|---------------|
| 50 | 1,119,155 | Hartogs        | ----- | Dec. 1, 1914  |
|    | 1,456,781 | Kessler et al. | ----- | May 29, 1923  |
|    | 1,906,041 | Barthelemy     | ----- | Apr. 25, 1933 |
|    | 1,920,188 | Dickie et al.  | ----- | Aug. 1, 1933  |
| 55 | 2,075,027 | Dreyfus        | ----- | Mar. 30, 1937 |
|    | 2,075,430 | Dreyfus        | ----- | Mar. 30, 1937 |